

No. 633,350.

Patented Sept. 19, 1899.

O. M. THOWLESS.

BURNER FOR INCANDESCENT LAMPS.

(Application filed July 23, 1898. Renewed Feb. 17, 1899.)

(No Model.)

Fig. 1.



Fig. 2.



Fig. 3.



WITNESSES:

Frank S. Ober  
Adam Frank

INVENTOR  
Orlando M. Thowless  
BY  
Albert Stevens  
ATTORNEY

# UNITED STATES PATENT OFFICE.

ORLANDO M. THOWLESS, OF NEWARK, NEW JERSEY.

## BURNER FOR INCANDESCENT LAMPS.

SPECIFICATION forming part of Letters Patent No. 633,350, dated September 19, 1899.

Application filed July 23, 1896. Renewed February 17, 1899. Serial No. 705,858. (No model.)

*To all whom it may concern:*

Be it known that I, ORLANDO M. THOWLESS, a subject of the Queen of Great Britain, and a resident of Newark, county of Essex, 5 State of New Jersey, have invented certain new and useful Improvements in Burners for Incandescent Lamps, of which the following is a specification.

My invention relates to incandescent lamps and burners for the same in which a thin strip of filament of highly-resisting material is caused to glow or incandesce by reason of the heat developed when a current of electricity is forced through said burner or filament. Hitherto such burners or filaments have been made of solid strips of carbon or other highly-resistant materials, and in some lamps metallic burners have been used. Hollow carbon-tube burners have also been employed. These lamps have, however, generally been of low efficiency and in most instances short-lived.

The object of my invention is to furnish a burner or filament which while being cheaply constructed is very efficient—that is, requiring few watts of energy per candle-power—and is more durable than any other with which I am acquainted.

The globe, the sealing, the exhaustion, the leading-in wires are the same as are generally employed in lamps of the incandescent class and require no further description.

To carry my invention into effect, I can proceed in various ways, which I will now describe.

The accompanying drawings show the general plan of my burner in its various forms. The burner is shown partly in section and partly in elevation.

Figure 1 shows the burner having an internal or basic filament; Fig. 2, a hollow non-conducting base without the internal filament, and Fig. 3 shows the non-conducting base as solid.

Referring to Fig. 1, A represents a burner composed of the internal filament B, the non-conducting base C, and the coating or deposited surface D.

Fig. 2 shows a burner A', composed of the hollow non-conducting base C' and the light-giving coating D'.

Fig. 3 shows the burner A'', composed of the solid non-conducting base C'', coated by the light-giving surface D''.

I take an ordinary incandescent lamp filament or burner or a metallic or composition wire and cover it with a non-conducting substance. For this basic filament I prefer to take a combination of carbon and alumina, carbon and iron, carbon and manganese, carbon and tungsten, or a metal or metallic compound or oxid having the property of forming conductors. One method of producing this non-conducting covering on the basic filament is to take, say, a cotton braid, soak it in a proper salt—for instance, nitrate of alumina—and apply it to the above-mentioned filament or burner. The burner thus covered is submitted to a high degree of heat, electric or otherwise, and the result is the destruction of the cotton covering, leaving a filament or burner covered with a so-called "non-conducting" material. (The word "non-conducting" is used in this specification in its usual electrical meaning—that is, a comparatively poor conductor). In order to deposit upon the non-conducting covering a layer of conducting material, the burner is then subjected to the process known in the art as "flashing." This is done by placing the burner thus prepared in the flashing jar or apparatus and exhausting the air from the same. When the air in the apparatus has reached the required degree of exhaustion, the air-pump is shut off and the flashing apparatus is filled with a hydrocarbon or other suitable gas. An electric current is then sent through the burner and the same is raised to a high degree of temperature, when the carbon from the gas begins to deposit upon the burner, and this operation is continued until the desired homogeneity and the required resistance of the burner is secured. After this has been accomplished the original or basic filament or substratum may be either removed by pulling it out, or chemically, or by burning it out with a heavy current, or by any other of the well-known methods. This removing of the substratum is not, however, absolutely necessary, as it may remain and assist in giving rigidity to the burner. I can, of course, also perform the flashing operation

by immersing the burner in a heavy hydro-carbon oil and heating it by means of an electric current.

There are other methods besides using cotton braid saturated with the appropriate salt by which I may secure the non-conducting material upon which the conducting-surface is deposited or coated. For instance, I may make a paste of the non-conducting material and apply it to the basic filament by means of a brush, or I may apply it chemically or by electric or igneous fusion or otherwise. The conducting-envelop of the burner may be simply drawn on over the non-conducting basic filament, like a hood, and be mechanically and electrically independent of the non-conducting portion, the latter serving merely to give shape and stability to the light-giving portion. In this construction the materials for the light-giving portion, the non-conducting basic filament, and the method of their treatment remain the same.

As materials for forming the non-conducting portion of the burner I have tried and recommend the nitrate, the sulfate, the chlorid, and the silicate of alumina, magnesia, and other similar substances whose salts when properly treated form a highly-resistant material. There are certain substances that I can use which under the combined reducing effect of heat and carbon may form carbids which, although comparatively poor conductors, would still be better conductors than some of the materials mentioned for the non-conducting covering. Such carbid-forming substances are, for instance, zirconium, thorium, calcium, silicon, and others. Although these carbids would not be so efficient as the layer of non-conducting material mentioned above, yet in some cases they may answer the purpose of the non-conducting covering.

Instead of using deposited carbon as the light-giving material I may deposit other substances answering the same purpose, for instance, metallic deposits, as metallic zirconium, niobium, molybdenum, or silicon; also, besides carbids mentioned above, some metallic oxids, as well as other materials that form conductors and are capable of being deposited or coated on the non-conducting base.

As I have said above, it is not necessary to remove the basic filament, but when it is left in order to give stability to the burner it does not form the light-giving portion of the burner, the electrical connection being made to the material deposited or coated upon the non-conducting portion of the burner.

In order to prepare the non-conducting base for receiving the carbon deposit in the flashing-jar when no internal filament is employed, I proceed as follows: I pour oil of rosemary on dry chlorid of platinum in a porcelain dish and knead it until all parts of it are well moistened. I then rub this up with five times its weight of oil of lavender and allow it to stand a short time in order to clear.

The filamentary strips are thinly coated with the above preparation and afterward heated in a muffle or over a Bunsen burner. This gives a coating of platinum to the surface 70 of the filament, which can then be placed in the hydrocarbon flashing-jar and carbon deposited thereon to the proper thickness.

For high-voltage lamps in which a very high resistance is necessary, I may employ 75 for the light-giving portion (deposited or coated) a conducting substance combined or mixed with a non-conducting or poorly-conducting one. For instance, a proper mixture of carbon and magnesia or of carbon and a 80 carbid may be deposited or coated upon the non-conducting portion of the burner and serve as the light-giving substance.

My invention is not limited in its scope to a strip or filamentary form, but may be applied to burners of any desired shape or size. For instance, the burners may have the form of a mantle or hood, such as is usual in the Welsbach or Auer gas-burner, or it may be button-shaped or in the form of a thin ribbon. 90

What I claim is—

1. A burner for incandescent or glow lamps composed of an internal basic filament or strip covered with a layer of non-conducting material and a light-giving surface deposited 95 thereon.

2. A burner for an incandescent lamp composed of a basic non-conducting filament having a loosely-fitting conducting-covering, designed to serve as the light-giving portion of 100 the burner.

3. The method of making burners for incandescent lamps, which consists in properly preparing the surface of an internal non-conducting core, solid or hollow, for receiving a 105 layer of electrically-deposited carbon, and then submitting the burner so prepared to the action of the flashing or other similar process.

4. A burner for incandescent lamps, consisting of a hollow tube or cylinder of non-conducting substance covered with a layer of 110 conducting material.

5. A burner for incandescent lamps, composed of a hollow internal filament or strip, a coating of non-conducting substance, and a 115 layer thereon of conducting material.

6. A burner for incandescent lamps composed of a properly-prepared non-conducting base, and having for its light-giving portion a composite material composed of a mixture 120 of conducting and poorly-conducting substances.

7. A burner for incandescent lamps, composed of an internal filament, a layer of non-conducting substance, and a covering of composite conducting material. 125

8. A burner for incandescent lamps, composed of a hollow non-conducting base covered with a layer of composite material formed of a mixture of conducting and non-conducting 130 substances.

9. A burner for incandescent lamps hav-

ing a properly-prepared internal non-conducting base, upon which is deposited or coated a light-giving portion of metallic carbid.

10. A burner for incandescent lamps, having a properly-prepared internal non-conducting core, and whose light-giving portion is composed of conducting metallic oxids.

11. The method of making burners for incandescent lamps, which consists in treating a chlorid of platinum with proper essential oils, applying the resultant compound to a non-conducting basic filament, heating the fila-

ment thus covered, and subjecting the filament thus formed to the action of an electric current in the presence of a hydrocarbon gas 15 or liquid.

In testimony that I claim the foregoing as my invention I have signed my name in presence of two witnesses.

ORLANDO M. THOWLESS.

Witnesses:

ADAM FRANK,  
JNO. J. FLYNN.